

April 11, 1939.

L. S. M. LEJEUNE

2,153,964

MANUFACTURE OF ELASTIC FABRIC

Filed Sept. 2, 1936



Inventor:-  
Leon Sylvain Max Lejeune  
By Mauro & Lewis,  
Attorneys.

## UNITED STATES PATENT OFFICE

2,153,964

## MANUFACTURE OF ELASTIC FABRIC

Leon Sylvain Max Lejeune, Paris, France, assignor, by mesne assignments, to Hevaloid Corporation, Dover, Del., a corporation of Delaware

Application September 2, 1936, Serial No. 99,159.  
In France, Great Britain, Ireland, and Mexico  
July 20, 1933

24 Claims.

(Cl. 28—1)

My present invention has for its object the manufacture of fabrics and products obtained therefrom, which are made from linear elements, such as described in the copending application 5 Serial No. 99,149 filed on Sept. 2, 1936, and which are woven and treated in such a manner as to be highly impregnable by liquids and which possess after impregnation extremely high qualities of elasticity and strength. My present application is a continuation-in-part-application of my 10 prior application Serial No. 735,314 filed July 16, 1934, and contains not only matter disclosed in said prior application, but also new improvements relating thereto.

15 It is known that the impregnation of fabrics by means of elastic or plastic material or other analogous materials becomes increasingly difficult as the fibres of the fabric are more tightened against one another, either from the beginning 20 by reason of the high initial twist of the thread or subsequently by the manner in which the fabric is made, or finally by the swelling of the threads at the time of impregnation, or by several of these causes acting at the same time. 25 Moreover the fabrics formed of threads already impregnated are difficult to make and it is necessary to re-impregnate the fabric if it is desired that its threads shall be well agglomerated together.

30 Fabrics made under normal conditions by means of special inverse twists such as those described in patent application Serial No. 99,149 of Sept. 2, 1936, above mentioned, are much superior in respect to impregnation, strength and 35 elasticity, but during the operation of swelling and contraction a certain compression is produced which often causes defective impregnation.

A fabric made of ordinary threads, that is to 40 say threads having a high twist and which are woven openly so as to have, after a swelling and contracting operation, the texture of a closely woven fabric, cannot be practically impregnated with elastic or plastic materials, even if the mesh 45 was initially so large that there was no supplementary transverse compression of the thread by reason of the contraction of the mesh. The thread forming such fabrics would have undergone, during the operation of swelling and contraction, a compression of its own, independent 50 of the shrinking of the mesh which compression would strongly oppose the penetration of the elastic or plastic material. To this compression there would be added that due to the swelling 55 of the threads under the effect of the vehicle

of the impregnating bath. Such a fabric moreover would not possess any substantial degree of elasticity.

The present invention on the contrary makes possible the production of fabrics very readily 5 and under normal conditions of weaving and impregnation which are both highly elastic and are also impregnated to the core in a single impregnating operation; and the invention embraces both the products, and also the process 10 whereby they are manufactured.

The manufacture of such readily impregnated fabrics according to the invention is rendered possible first of all by the fact that the fabric is constituted not with ordinary threads, but 15 with the special linear elements so called "inverse twists", described in the copending application Serial No. 99,149, which are formed each of a plurality of rovings which have been supertwisted individually in one direction to 20 such an extent that they cannot be substantially drawn out, and which have been then assembled together by a twisting in the opposite direction for approximately the same number 25 of turns as that of the individual twist of each roving.

The process according to the invention is essentially characterized in that, with the said special open linear elements whose fibres do not exert appreciable mutual compression, an open-mesh fabric loosely woven is made, the degree of opening of the linear elements and the initial dimension of the mesh of the fabric being such that, when the fabric is submitted to a swelling and contracting operation without tension by 30 means of an agent such for example as a strong acid or a strong base, the linear elements remain open and approach one another without the said open elements being appreciably compressed.

In the operation of swelling and contracting the closing up increases, that is to say the difference between the extended length of the linear element and its apparent length in warp and weft becomes greater. Once this swelling 45 and this contraction without tension and without compression are effected, there is attained a fabric having a greater strength and elasticity than originally, and which can be used in place of ordinary fabrics.

The size of the mesh to be chosen before treatment obviously depends on the nature and size of the linear elements used as well as on the degree of swelling and contraction which the elements are destined to undergo. The num- 50 55

ber of linear elements to the centimetre should obviously always be proportioned to the nature of the element and to the swelling and contracting treatments.

5 In order to make fabrics of considerable thickness, it is of advantage to weave bundles of "inverse twists" into a loose mesh fabric, that is to say, bundles each formed of a plurality of "inverse twists", so that the linear element 10 constituted by one such bundle has the desired thickness.

It is to be noted that, instead of employing a plain weave, it may be of advantage to arrange the layers of inverse twists as a sateen 15 weave.

15 The swelling and contracting agents for treating the loose mesh fabric may be such as are usually employed (strong acid or strong base) which are capable of transforming more or less 20 completely the cellulose into hydrocellulose without harming it; for example, good results are obtained by treating the loose-mesh fabric with caustic soda of 30° Bé. at 18° C. for about 15 minutes.

25 The first operation performed on the loose-mesh textile fabric consists in treating it without tension by means of a strong swelling and contracting agent such as soda.

30 In carrying out the contracting and swelling treatment it may be useful to employ a wetting agent, in order that the loose-mesh fabric be fully wetted by the bath in which it is immersed. As wetting agent may be employed any wetting agent which is commonly known for the usual 35 treatments of textiles with liquids.

40 The fabric is allowed to remain in the bath under the conditions described which are such that a close-mesh fabric is obtained in which however no substantial compression between the linear elements and between their fibres takes place; afterwards the fabric is removed from the bath and is expressed so that the greater part of the bath may be recovered.

45 Preferably, after having been subjected to the treatment with the bath of contracting and swelling agent, and having been carefully washed, the fabric according to the invention is subjected to a boiling treatment, which is carried out under the conditions usual for such a treatment in the textile industry, for example with the aid of carbonate of soda lye, at the high temperature convenient for boiling.

50 The boiling treatment may be carried out as follows: the fabric, carefully washed, is given a boiling by means of a lye of carbonate of soda of 3%, to which there is added a soda soap of 1.5% under a pressure of 1.5 atm. corresponding to a temperature of 113° C. for 4 hours. The percentage is calculated always with respect to the 55 weight of dry cotton.

55 After such boiling treatment, the fabric preferably is washed with warm water, then with cold water, and afterwards is treated with hydrochloric acid or the like, then is washed anew and 60 finally is carefully dried. As an example of such treatment subsequent to boiling, the fabric after boiling may be washed with warm water at 90° for about 1 hour, carefully washed with cold water, neutralized through a solution of commercial 65 hydrochloric acid of 0.5° Bé., then again washed till the chlorides are eliminated. Finally the treated fabric is carefully dried so that there remains only about 7% of wetness with respect to the weight of the dry cotton. The fabric is 70 then ready for impregnation. One of its essen-

tial characteristics is that it is very easily impregnated, due to the fact that the linear elements forming it are very open and not appreciably compressed against each other.

75 To make a rubberized fabric according to the invention the tensile strength required is first considered at the same time as the thickness required for the fabric. There is taken for example a linear textile element consisting of a special non-treated inverse twist such as defined above 10 and corresponding to the diameter required; then a fabric is made having a texture in warp and weft 50% inferior in strength to that required in the ultimate product. The fabric is then subjected to the treatment above described of 15 contracting and swelling, of boiling, washing and drying and then the acquired properties of the fabric are fixed by impregnation with rubber latex. If the impregnation is to take place by 20 means of a solution of rubber or other like impregnating material, drying is performed before impregnation; otherwise it is not necessary to dry it until after impregnation.

25 The fabric obtained after the successive treatments described above being highly impregnable, in order to impregnate it with elastic or plastic material (rubber, balata, or other materials of the same kind) derived either from latex or from a solution of rubber in a volatile solvent, the impregnation may be performed in any known manner but without exercising tension or compression upon the fabric; for example by simple 30 immersion in a natural or artificial suspension of elastic or plastic material, such as rubber latex or even in a solution of these materials in a volatile solvent. Obviously rinsings and dryings which would normally be necessary between the several operations will be performed. As afore 35 said, the impregnation fixes the properties of the fabric, particularly its strength and elasticity. 40

45 Preferably the impregnation is carried out by immersion of the fabric in a bath of latex, containing for example 40% of dry rubber with the vulcanising agents. The impregnation occurs preferably without vacuum or pressure being applied, in vats or other receptacles which are closed with a cover which is sufficiently tight to prevent evaporation of the ammonia, which would result in the coagulation of the surface of the bath. After each impregnating operation 50 the ammonia content of the bath is brought to the required degree by adding thereto a solution of commercial ammonia.

55 After the impregnation, the fabric is placed in conditions suitable for coagulating the rubber. To effect this, the ammonia is allowed to evaporate or is neutralized.

60 When the coagulation is effected, the impregnated fabric is placed in such conditions that the greater part of the water still contained therein evaporates. To effect this, the fabric can be calendered with an ordinary calender so as to remove therefrom as much water as possible. Afterwards the product is dried in any suitable manner. Care should be taken that the temperature of the drying apparatus be lowered as 65 the fabric dries.

70 The quantity of water remaining at that time in the fabric will not exceed preferably 4% of the weight of the impregnated fabric.

75 In most cases, the impregnating treatment is followed by vulcanization. The fabric when impregnated is preserved until it is desired to vulcanize the same, and for this purpose is kept preferably in warehouses which are dimly lighted

and not too damp. When it is desired to obtain fabrics composed of several plies or thicknesses, the component plies are to be stuck together prior to warehousing in order to prevent oxidation of the surfaces of the plies.

If it is desired to deprive the fabric thus impregnated of part of its natural property of elongation it is stretched in the direction in which it is desired to limit the elasticity, the degree of stretching being such that the fabric is brought to the desired degree of elongation. Then the fabric is vulcanised under this tension thereby fixing the dimensions of the fabric and at the same time the lower limit of its elasticity. This fixation may also be effected by the same means during the operation of drying: Due to the very great inherent elasticity of a fabric thus made it is possible to approach the initial dimensions of the fabric before treatment while conserving an appreciable residual elasticity. Obviously if desired the elasticity may be caused completely to disappear and the dimensions of the completed fabric be made equal to or even greater than its initial dimensions.

25 The product is vulcanized, preferably under a pressure of about 25/30 kg. per cm<sup>2</sup>.

The present invention also comprises means for preventing any substantial bulging or warping of the fabric due to the fact that the selvages of the same are always more compressed than the rest of the fabric. In order to avoid any risk of such bulging, it is preferred, before the operation of stretching and vulcanization, to cut the selvages of the fabric in such a manner that the strips or sheets finally obtained are prevented from bulging. As aforesaid, the removal of the selvages by cutting should take place before the fabric is stretched.

40 Fabrics impregnated according to this invention may be used industrially for all purposes for which impregnated fabrics are normally used, notably for tires, belts, tarpaulins, impermeable fabrics for clothes, flexible pipes etc.

The invention is illustrated by way of example 45 in the accompanying drawing, in which:

Figure 1 shows schematically on a large scale a section of an ordinary fabric of close weave, as heretofore made;

Figure 2 shows a fragment of the same fabric 50 after increase of the diameter of the warp threads only, the weft threads being assumed to have been able to spread and slide freely with respect to the warp threads, these latter being consequently regarded as able to move apart freely from one another;

Figure 3 shows the same schematic fabric after 55 increase of the diameter not only of the warp threads but likewise of the weft threads, the warp threads being regarded as free to move apart again without resistance and the weft threads as being able to slide freely with respect to the warp threads;

Figure 4 is a face view, likewise schematic, on a smaller scale of a fragment of fabric after the 60 first operation of manufacture according to this invention;

Figure 5 is a section on line A—A of Figure 4;

Figure 6 is a schematic view on the same scale as Figures 4 and 5, showing the same fabric 65 after the operation of swelling of the twisted elements of the warp and weft;

Figure 7 is a section of the same fabric on line B—B of Figure 6 after the swelling operation.

If a close fabric is formed such as that shown 70 in Figure 1 and which comprises linear weft ele-

ments 1a, 1b and linear warp elements 2a, 2b, tightly woven, and if such a fabric is treated so as to cause the diameter of the linear warp elements and the linear weft elements to increase, the linear weft elements will become 1'a, and 5 1'b (Figure 3) and the linear warp elements 2'a, 2'b (Figures 2 and 3) assuming that they have been able to swell and to slide freely. But as in practice the weft and warp threads cannot slide freely, the fabric will tighten and there will result from this a compression of the linear elements composing it; the result being that not only will the fabric have no more strength and elasticity than it had initially, but also the fabric, being tightened instead of opening, the rubber 10 cannot penetrate it for the purpose of fixing the properties of the fabric.

If on the contrary, according to this invention, there is formed a fabric such as shown in Figures 4 and 5 by starting from a very open 20 linear textile element, i. e. a special "inverse twist," (weft linear elements 1a, 1b, warp linear elements 2a, 2b) such that when the fibres are swollen and contracted without tension they are not compressed, said fabric being formed of large 25 mesh,—meshes of such size that when the swelling and contraction are produced there will result, without perceptible compression of the warp and weft linear elements, a fabric like that shown in Figures 6 and 7 (weft linear elements 1'a, 1'b, 30 warp linear elements 2'a, 2'b)—and if then the fabric of Figures 4 and 5 is transformed into that of Figures 6 and 7 by the swelling and contracting operation, a fabric will have been formed in which the closing up will have been considerably increased but which, by reason of the absence of compression of the linear elements which compose it, will be able very readily to absorb an elastic or plastic material without decrease 35 either of the strength or the elasticity of the 40 fabric, the impregnation having on the contrary the effect of fixing its properties of elasticity and tensile strength and those of cohesion of the elements which compose it. In practice the linear elements will be deformed in a certain measure 45 in the transverse direction and their cross section will not remain exactly the same; but, given the fact that the initial linear element is very open and very deformable transversely and that on the other hand the fabric has been woven 50 with very loose meshes and moreover that the swelling and the contraction have taken place without tension, the deformation which the linear elements will have undergone will take place without the fibres being compressed against one another. The linear element will spread for example at the crossing points of the fabric without sensibly increasing the pressure of the fibres 55 upon each other.

As a non-limiting example, one may start with 60 a linear element constituted by a special inverse twist such as defined above of No. 14/2 American cotton, formed of two rovings twisted individually 480 turns per metre to the right, then assembled and twisted together 480 per metre in the reverse direction. With this twist there will be formed a square cloth fabric having 9 warp threads and 65 9 weft threads per centimetre, which fabric will then weigh 150 grams per metre. For a band of 70 5 centimeters in width such a fabric has a strength at breaking of 37 kgs. It has a total elongation at breaking of 20% and practically no residual elasticity. (The residual elasticity 75 is the real elasticity which exists after an initial

non-elastic elongation in which the fibres have assumed their position of equilibrium.)

This fabric is treated with a caustic soda lye of 30° Bé. at a temperature of 18° C. for 15 minutes. The fabric swells and contracts but the warp and weft threads—due to the fact that the treatment is effected without tension and also that the fabric had very open meshes—are not substantially compressed although the fabric has become a tight textured fabric, that is to say whose threads are close together. This new fabric weighs 300 grams per square metre and it has in warp and weft 14 warp threads and 14 weft threads per centimetre. With a strip having a width of 5 centimetres it has a breaking strength of 62 kgs., 40% elongation and 30% residual elasticity.

The swelling and the contraction of the threads are 30% in warp and weft. There are 14—9=5 more threads per centimetre, or 55% increase. The weight has become 150 grams plus 55% of 150 grams=150+82 grams=232 grams, no account being yet taken of the swelling and shortening of the warp and weft. The swelling of 30% of the warp and weft calculated upon 232 grams results in an increasing of the weight

$$=232 \times 30\% = 69 \text{ grams,}$$

making a total of 232 grams+69 grams=301 grams which corresponds to within a gram of the figure stated above resulting from physical tests.

Then the fabric is subjected to the treatment of boiling, washing, neutralizing, anew washing and drying as has been described above, and finally to impregnation.

After rubbering by means of latex and after vulcanization the fabrics had 75 kg. strength at breaking upon a band of 5 cm. width and 50% of entirely residual elasticity, the strength and the elasticity being fixed at these figures by the rubber of the impregnation.

It is to be noted that in all cases, given the normal conditions required, it is possible to attain the desired conditions by a preliminary calculation. Supposing that the conditions required are 75 kgs. tensile strength in bands of 5 cm. and 0.5 mm. thickness, after impregnation one will take for example a 14/2 linear element. Its diameter D being calculated by the known method

$$D = \frac{L}{n}$$

(L being the length and n the number of spirals) a diameter of  $D=0.4$  mm. will be found. Given that it is possible to obtain by a treatment with soda with a concentration, temperature and duration, such as have been given above, a swelling of 30%, it will be realized that one may reckon upon a final diameter  $D=0.52$ .

The warp and weft being superposed upon one another, for thickness of the fabric one will have 0.52 mm. multiplied by 2=1.04 mm. but taking into account the inherent compressibility of the article and knowing by experience that one can count on being able to reduce the thickness by 50% by a subsequent compression of the assembly of the fabric after impregnation, this will permit a final thickness of

$$\frac{1.04}{2} \text{ mm.} = 0.52 \text{ mm.}$$

the thickness required. This compression will not harm in any manner the fibres of the fabric

because of the absence of compression of the fibres of the fabric during its manufacture.

The 14/2 thread of American cotton has a tensile strength of about 700 grams. The strength of each thread being increased by 50% by the treatment mentioned above, there is obtained for each thread a tensile strength of 1050 grams. One should thus have in mind for the number of threads to the centimetre

$$\frac{75}{1.050} \text{ kgs.} = 71$$

threads for a band of 5 cm. or 14 threads per cm.

As the fabric increases by 50% in number of warp and weft threads by the swelling and contracting treatment of 30%, the initial fabric should be formed with 9 warp and 9 weft threads.

The swelling and the contraction of 30% produced by the operation effected in the conditions stated above will thus result in a fabric with 14 warp and 14 weft threads per cm. This fabric will then be rubbered as has been stated above by impregnation, drying, regulation of the residual elasticity, if desired, and compression to the desired thickness and vulcanization.

In the preceding descriptions reference has been generally made to rubber, but it is obvious that analogous results would be obtained with elastic or plastic materials such, for example, as balata or other similar elastic or plastic substances.

The fabrics according to the invention are, by reason of their strength and elasticity, adapted to the manufacture of pneumatic tires.

For the manufacture of power transmission belts, fabrics according to the invention may be employed in the manner customarily used for the fabrication of those articles. However, the great elasticity of the fabric and the facility of fixing its residual elasticity, and on the other hand the fact that it is necessary to have in the transverse direction of the belt only ever so little elasticity, make it possible to manufacture, with the fabric according to the invention, belts which possess almost no transverse elasticity while having a high longitudinal elasticity.

For this purpose the fabric is caused to undergo after rubbering, such a tension in the transverse direction of the belt (weft of the fabric) that the elasticity of the fabric disappears and that the fabric is brought back to its original width or even to a larger width. Then the fabric is dried and its elastic properties are thus regulated. After drying the fabrics are assembled by the known processes in sufficient number of plies for obtaining the desired thickness. This assembly of fabrics is then pressed and vulcanised. Before pressing one may, if desired, regulate the elasticity in the direction of warp as has been described above.

For the manufacture of fabrics for clothing and other analogous applications, one will regulate preferably without any tension the elasticity which is in this case a fundamental element.

What I claim is:

1. A process for the manufacture of elastic fabric comprising the steps of forming linear textile elements very open throughout to penetration by liquids and substantially without reciprocal compression between the constituent fibres, weaving said elements into a fabric having meshes of such dimensions that when treated with a strong contracting and swelling agent a close mesh fabric is formed without however

transversely compressing said linear elements appreciably, and then treating said fabric with a suitable contracting and swelling agent.

2. In the manufacture of elastic fabric forming linear elements composed of rovings that have been supertwisted a certain number of turns without substantial tension in one direction and assembled by being twisted approximately the same number of turns in the opposite direction,

10 weaving said elements into a fabric having meshes of such dimensions that when treated with a strong contracting and swelling agent a close mesh fabric is formed without however compressing said linear elements appreciably, and then treating said fabric with a suitable

15 contracting and swelling agent.

3. Process for the manufacture of elastic fabric comprising the steps of forming very open linear elements substantially without reciprocal com-

20 pression between the constituent fibres thereof by individually supertwisting a plurality of rovings without substantial tension a certain number of turns in one direction and assembling them by twisting them approximately the same num-

25 ber of turns in the opposite direction, forming said linear elements into a fabric having large meshes, and treating said fabric with a strong contracting and swelling agent until the linear elements are brought close together without ap-

30 preciable compression thereof.

4. Process for the manufacture of elastic fab- ric comprising the steps of forming linear tex-

35 tile elements very open throughout to penetra-

tion by liquids and substantially without re-

40 ciprocal compression between the constituent fibres, weaving said elements into a fabric hav-

ing meshes of such dimensions that when treated with a strong contracting and swelling agent a close mesh fabric is formed without however

45 compressing said linear elements appreciably, then treating said fabric with a suitable con-

50 tracting and swelling agent, and then impreg- nating it with an elastic material.

5. Process for the manufacture of elastic fab-

55 ric comprising the steps of forming linear ele-

60 ments composed of rovings that have been super-

65 twisted a certain number of turns without sub-

70 stantial tension in one direction and assembled by being twisted approximately the same number of turns in the opposite direc-

75 tion, thereby forming open linear elements sub-

stantially without reciprocal compression be-  
tween the constituent fibres thereof, forming  
said linear elements into a fabric having large  
meshes, treating said fabric with a strong con-  
tracting and swelling agent until the linear ele-  
ments are brought close together without appre-  
ciable compression thereof, and impregnating  
said fabric with an elastic material.

8. Process for the manufacture of elastic fab-  
ric comprising the steps of forming open linear 10  
elements substantially without reciprocal com-  
pression between the constituent fibres thereof,  
forming said elements into a fabric having large  
meshes, treating said fabric with a strong con- 15  
tracting and swelling agent until the linear ele-  
ments are brought close together without appre-  
ciable compression thereof, impregnating said  
fabric with a vulcanizable material and vul-  
canizing the same.

9. Process for the manufacture of elastic fab- 20  
ric comprising the steps of forming open linear  
elements substantially without reciprocal com-  
pression between the constituent fibres thereof,  
forming said elements into a fabric having large  
meshes, and treating said fabric with a strong 25  
contracting and swelling agent until said linear  
elements are brought close together without ap-  
preciable compression thereof and the cellulose  
of their component fibres is converted into hydro-  
cellulose, and impregnating said fabric with an 30  
elastic material.

10. Process for the manufacture of an elastic  
fabric which consists in forming open linear ele-  
ments substantially without reciprocal compres-  
sion between the constituent fibres thereof, form- 35  
ing said elements into a fabric having large  
meshes, treating said fabric with a strong con-  
tracting and swelling agent until the linear ele-  
ments are brought close together without ap-  
preciable compression thereof, impregnating the 40  
fabric with an elastic material and drying the  
impregnated fabric under tension.

11. A process for the manufacture of elastic  
fabric comprising the steps of forming linear 45  
textile elements very open throughout to pene-  
tration by liquids and substantially without re-  
ciprocation compression between the constituent  
fibres, weaving said elements into a fabric hav-  
ing meshes of such dimensions that when treated 50  
with a strong contracting and swelling agent a  
close mesh fabric is formed without however  
transversely compressing said linear elements ap-  
preciable, then treating said fabric without ten-  
sion with a suitable contracting and swelling 55  
agent added with a wetting agent, and subject-  
ing said fabric to a boiling treatment, to washing  
and drying.

12. In the manufacture of elastic fabric form-  
ing linear elements composed of rovings that, 60  
have been super-twisted a certain number of  
turns without substantial tension in one direc-  
tion and assembled by being twisted approxi-  
mately the same number of turns in the oppo-  
site direction, weaving said elements into a fabric 65  
having meshes of such dimensions that when  
treated with a strong contracting and swelling  
agent a close mesh fabric is formed without how-  
ever compressing said linear elements appreci-  
ably, and then treating without tension said fab- 70  
ric with a suitable contracting and swelling agent  
added with a wetting agent, and subjecting said  
fabric to a boiling treatment, to washing and  
drying.

13. Process for the manufacture of elastic fab-  
ric comprising the steps of forming very open 75

- linear elements substantially without reciprocal compression between the constituent fibres thereof by individually supertwisting a plurality of rovings without substantial tension a certain 5 number of turns in one direction and assembling them by twisting them approximately the same number of turns in the opposite direction, forming said linear elements into a fabric having large meshes, and treating said fabric until the 10 linear elements are brought close together without appreciable compression thereof with a strong contracting and swelling agent added with a wetting agent, and subjecting said fabric to a boiling treatment, to washing and drying.
15. 14. Process for the manufacture of elastic fabric comprising the steps of forming linear textile elements very open throughout to penetration by liquids and substantially without reciprocal compression between the constituent fibres, weaving said elements into a fabric having meshes of such dimensions that when treated with a strong contracting and swelling agent a close mesh fabric is formed without however compressing said linear elements appreciably, then treating said 20 fabric with a suitable contracting and swelling agent added with a wetting agent, and subjecting said fabric to a boiling treatment, to washing and drying and then impregnating it with an elastic material.
30. 15. Process for the manufacture of elastic fabric comprising the steps of forming linear elements composed of rovings that have been supertwisted a certain number of turns without substantial tension in one direction and assembled 35 by being twisted approximately the same number of turns in the opposite direction, weaving said elements into a fabric having meshes of such dimensions that when treated with a strong contracting and swelling agent a close mesh fabric 40 is formed without however compressing said linear elements appreciably, then treating said fabric with a suitable contracting and swelling agent added with a wetting agent, and subjecting said fabric to a boiling treatment, to washing and drying and 45 impregnating it with an elastic material.
16. Process for the manufacture of elastic fabric comprising the steps of forming very open linear elements substantially without reciprocal compression between the constituent fibres thereof, forming said elements into a fabric having large meshes, treating said fabric until the linear elements are brought close together without appreciable compression thereof with a strong contracting and swelling agent added with a wetting agent, and subjecting said fabric to a boiling treatment, to washing and drying and impregnating said fabric with an elastic material.
17. Process for the manufacture of elastic fabric comprising the steps of individually supertwisting a plurality of rovings without substantial tension a certain number of turns in one direction and twisting them together approximately the same number of turns in the opposite direction, thereby forming open linear elements substantially without reciprocal compression between the constituent fibres thereof, forming said linear elements into a fabric having large meshes, treating said fabric until the linear elements are brought close together without appreciable compression thereof with a strong contracting and swelling agent added with a wetting agent, and subjecting said fabric to a boiling treatment, to washing and drying and impregnating said fabric with an elastic material.
18. Process for the manufacture of elastic fabric comprising the steps of forming open linear elements substantially without reciprocal compression between the constituent fibres thereof, forming said elements into a fabric having large 5 meshes, treating said fabric until the linear elements are brought close together without appreciable compression thereof with a strong contracting and swelling agent added with a wetting agent, and subjecting said fabric to a boiling 10 treatment, to washing and drying, impregnating said fabric with a vulcanizable material coagulating the same, drying it, cutting the selvages of the fabric so as to prevent the same from bulging, and subjecting the fabric to stretching and vulcanization.
19. Process for the manufacture of elastic fabric comprising the steps of forming open linear elements substantially without reciprocal compression between the constituent fibres thereof, 20 forming said elements into a fabric having large meshes, and treating said fabric with a strong contracting and swelling agent added with a wetting agent until said linear elements are brought close together without appreciable compression 25 thereof and the cellulose of their component fibres is converted into hydrocellulose, subjecting the fabric to a boiling treatment, to washing and drying and impregnating said fabric with an elastic material, coagulating the same and drying 30 it and cutting the selvages of the fabric so as to prevent the same from bulging.
20. Process for the manufacture of an elastic fabric which consists in forming open linear elements substantially without reciprocal compression 35 between the constituent fibres thereof, forming said elements into a fabric having large meshes, treating said fabric until the linear elements are brought close together without appreciable compression thereof with a strong contracting and swelling agent added with a wetting agent, then subjecting the fabric to a boiling 40 treatment, to washing and drying, impregnating the fabric with an elastic material and drying the impregnated fabric under tension.
21. An elastic textile product composed of textile linear elements very open throughout and substantially without reciprocal compression between the constituent fibres, said linear elements being formed into a fabric having meshes of such dimensions that they are in contact with each other without appreciably compressing each other and being thoroughly impregnated and united together by an elastic substance which fills the interstices between the constituent fibres and binds 50 them into a dense, strongly cohesive and highly compressible product.
22. An elastic textile product formed of fibrous linear elements composed of supertwisted rovings in a very open condition united by a twist in the reverse direction to that of the individual rovings which are substantially without reciprocal compression between the constituent fibres, said linear elements being formed into a fabric of such close weave that they are in contact with each other but without appreciably compressing 55 each other and being thoroughly impregnated and united together by an elastic substance which fills the interstices between the constituent fibres and binds them into a strongly cohesive and highly compressible product.
23. A thick elastic fabric formed of bundles of fibrous linear elements composed of supertwisted rovings in a very open condition united by a twist in the reverse direction to that of the in- 60

8 individual rovings which are substantially without reciprocal compression between the constituent fibres, said linear elements being formed into a fabric of such close weave that they are in contact with each other but without appreciably compressing each other and being thoroughly impregnated and united together by an elastic substance which fills the interstices between the constituent fibres and binds them into a strongly cohesive and highly compressible product.

10 24. An elastic textile product formed of fibrous linear elements composed each of two rovings of size 2.5 (French size), supertwisted so as to have each a total twist of about 200 turns in one direc-

tion and united by a twist of about 200 turns, so that there is no substantial compression between the constituent fibres, in the reverse direction to that of the individual twist, said linear elements being formed into a fabric of such close weave that they are in contact with each other but without appreciably compressing each other and being thoroughly impregnated and united together by an elastic substance which fills the interstices between the constituent fibres and binds them 10 into a strongly cohesive and highly compressible product.

LÉON SYLVAIN MAX LEJEUNE.